

1

3,127,265  
Ni-Cr-Co ALLOYS  
Howard S. Avery, Mahwah, N.J., assignor to American  
Brake Shoe Company, New York, N.Y., a corporation  
of Delaware  
No Drawing. Filed Aug. 8, 1961, Ser. No. 130,000  
3 Claims. (Cl. 75—171)

This invention relates to heat and corrosion resistant alloys for structural parts in industrial furnaces and like installations where structural parts must possess high resistance to oxidation in addition to exceptional levels of hot strength, and which can be cast or forged. This application is a continuation-in-part of application Serial No. 808,024, filed April 22, 1959, now abandoned.

For engineering applications involving elevated temperature service, the so-called creep characteristics of the alloy used for structural materials are frequently of major importance as well as oxidation and corrosion resistance characteristics. Thus, in such applications failure of structural parts can result from excessive creep (plastic deformation) as well as rupture under load due to external or internal deterioration caused by oxidation and corrosion occurring progressively inwardly of the part, as in the presence of hot corrosive flue gases. Engineering developments in the petro-chemical industry, in the manufacture of furnace equipment and in other high temperature industries are limited by the capabilities of available alloys. For example, there is need for oxidation-resistant alloys with high creep and rupture strengths in the temperature range of 1800° F. to 2300° F. For the cast industrial heat-resistant alloys (such as the Alloy Casting Institute grades) a few display reasonably good oxidation resistance up to 2150° F., but their strength is low. Some exceptional properties are reported with cobalt-base alloys having 55 percent or more cobalt, but these are expensive. In comparison, the cobalt content in the alloys of the present invention need not exceed

2

iron. It has heretofore been proposed to use as an addition one or more of molybdenum, titanium with aluminum, and columbium for enhancing the hot strength of such alloys. For one reason or another, these additions have rather serious drawbacks and therefore limit utilization of the resultant alloy. The titanium plus aluminum addition, for example, causes trouble with surface films and reacts with oxygen and nitrogen, and hence makes the alloy difficult to cast in the absence of special techniques such as vacuum melting or controlled atmosphere. Columbium and molybdenum individually tend to lessen resistance to oxidation at 2000° F., and hence life expectancy is lessened. Tungsten, on the other hand, seems to have none of these drawbacks, and appears to enhance the strength of the austenite matrix afforded by the nickel and chromium contents.

It is an object of the present invention to achieve hot strength characteristics in a heat and corrosion-resistant alloy of the nickel-base type but containing tungsten, and to do this by way of a limited cobalt addition, the preferred alloy of the present invention being further characterized by the absence of molybdenum, titanium and columbium.

Thus, in accordance with the present invention, it has been found that with tungsten present in a nickel base, heat-resistant alloy, life expectancy can be appreciably increased and minimum creep rate significantly lowered by adding cobalt. The data in Table I demonstrate the improvement, and here the variations in silicon, manganese, nickel, chromium and tungsten have no significant effect on hot strength data. Increasing carbon improves hot strength, and this is also true of optimum amounts of dissolved nitrogen. The balance for each alloy in Table I is substantially all iron, and this is also true of the other alloys disclosed herein in definite percentage amounts. The minimum creep rate is the minimum or so-called stage II creep rate of the standard constant temperature-constant load creep test.

TABLE I  
Properties of Cast Heat-Resistant Alloys at  
2000° F., 2500 p.s.i. Stress

| Heat No. | C    | Mn   | Si   | Ni   | Cr   | N     | W     | Co    | Life<br>(hrs.) | MCR <sup>1</sup> |
|----------|------|------|------|------|------|-------|-------|-------|----------------|------------------|
| 419----- | 0.63 | 0.97 | 1.10 | 34.7 | 28.1 | 0.105 | 4.65  | ----- | 114            | 0.063            |
| 477----- | 0.55 | 0.08 | 1.28 | 35.8 | 28.1 | 0.087 | 24.73 | ----- | 149            | 0.043            |
| 452----- | 0.54 | 0.10 | 1.27 | 35.7 | 23.4 | 0.086 | 24.77 | ----- | 94.8           | 0.039            |
| 17-----  | 0.50 | 0.04 | 1.39 | 35.2 | 23.0 | 0.109 | 24.35 | 15.05 | 783            | 4 0.0008         |

<sup>1</sup> Minimum creep rate-percent/hr.

<sup>2</sup> Zirconium, calcium and aluminum added as deoxidizers. Residual zirconium, 0.032%; residual aluminum 0.075%.

<sup>3</sup> Deoxidized with aluminum only; residual, 0.077%.

<sup>4</sup> Minimum values of 0.0003 and 0.0008 were obtained.

about 25 to 26 percent, and the present alloys are not cobalt base.

Heat and corrosion resistant alloys characterized by a nickel base and containing substantial amounts of chromium are known, and some include substantial amounts of

Exceptional values of minimum creep rate (MCR in Table II—percent per hour) were noted with the alloys in Table II at the indicated temperatures and under the indicated stress, and quite prolonged life (in hours) was obtained.

TABLE II.—HEAT RESISTANT ALLOYS

| Heat No. | Chemical Composition |      |      |      |      |      |      |       | Properties               |                  |                 |                          |                  |                 |                          |                  |                 |
|----------|----------------------|------|------|------|------|------|------|-------|--------------------------|------------------|-----------------|--------------------------|------------------|-----------------|--------------------------|------------------|-----------------|
|          | C                    | Mn   | Si   | Cr   | Ni   | Co   | W    | N     | 1800° F. and 8000 p.s.i. |                  |                 | 2000° F. and 2500 p.s.i. |                  |                 | 2200° F. and 1000 p.s.i. |                  |                 |
|          |                      |      |      |      |      |      |      |       | Life, hours              | MCR, percent/hr. | Elong., percent | Life, hours              | MCR, percent/hr. | Elong., percent | Life, hours              | MCR, percent/hr. | Elong., percent |
| 11       | 0.31                 | 0.24 | 0.99 | 25.5 | 26.3 | 25.2 | 15.1 | 0.07  | 374.9                    | 0.0046           | 6.0             | -----                    | -----            | -----           | -----                    | -----            | -----           |
| 12       | 0.35                 | 0.28 | 1.36 | 22.1 | 36.3 | 25.4 | 12.0 | ----- | 118.6                    | 0.014            | 5.5             | -----                    | -----            | -----           | -----                    | -----            | -----           |
| 13       | 0.42                 | 0.06 | 1.44 | 28.3 | 36.6 | 14.8 | 4.97 | 0.12  | 47.0                     | 0.139            | 23.0            | 674.9                    | 0.0021           | 11.0            | 105.7                    | 0.091            | 22.0            |
| 14       | 0.49                 | 0.17 | 1.51 | 28.1 | 40.9 | 14.8 | 4.89 | 0.11  | 57.9                     | 0.124            | 19.5            | 1,471.8                  | 0.00028          | 7.0             | 252.8                    | 0.0017           | 10.0            |
| 15       | 0.49                 | 0.11 | 1.39 | 28.0 | 36.2 | 18.3 | 9.05 | 0.10  | 78.1                     | 0.039            | 8.0             | 626.2                    | 0.00195          | 8.5             | 265.9                    | 0.0085           | 9.5             |
| 16       | 0.50                 | 0.08 | 1.47 | 28.2 | 36.4 | 9.80 | 4.85 | 0.10  | 26.3                     | 0.219            | 26.5            | 530.3                    | 0.0020           | 11.0            | 120.5                    | 0.009            | 11.5            |
| 17       | 0.50                 | 0.04 | 1.39 | 28.0 | 35.5 | 15.1 | 4.85 | 0.11  | 40.6                     | 0.074            | 20.0            | 782.7                    | 0.0008           | 6.2             | 207.2                    | 0.011            | 15.0            |
| 18       | 0.50                 | 0.13 | 1.47 | 28.2 | 36.4 | 15.3 | 4.99 | 0.10  | 81.7                     | 0.072            | 19.0            | 1,160.1                  | 0.00017          | 4.0             | 280.5                    | 0.0033           | 15.0            |
| 19       | 0.50                 | 0.08 | 1.47 | 28.2 | 36.5 | 14.6 | 4.94 | 0.11  | 42.0                     | 0.133            | 26.0            | 358.3                    | 0.00099          | 4.0             | 185.3                    | 0.104            | 44.0            |
| 20       | 0.50                 | 0.04 | 1.41 | 29.1 | 35.6 | 14.8 | 9.06 | 0.09  | 66.5                     | 0.073            | 12.0            | 535.1                    | 0.0075           | 20.0            | 218.2                    | 0.020            | 16.5            |
| 21       | 0.52                 | 0.09 | 1.28 | 28.1 | 39.8 | 13.7 | 8.90 | 0.10  | 73.7                     | 0.070            | 13.0            | 523.8                    | 0.0021           | 5.5             | 205.2                    | 0.0061           | 6.5             |
| 22       | 0.53                 | 0.29 | 1.32 | 31.9 | 38.2 | 20.4 | 6.95 | ----- | 50.0                     | 0.134            | 11.5            | -----                    | -----            | -----           | -----                    | -----            | -----           |
| 23       | 0.53                 | 0.06 | 1.50 | 28.3 | 36.8 | 19.2 | 4.92 | 0.11  | 79.8                     | 0.057            | 14.0            | 638.5                    | 0.0007           | 3.5             | 245.6                    | 0.0019           | 10.0            |
| 24       | 0.53                 | 0.07 | 1.28 | 25.8 | 37.8 | 19.7 | 7.13 | 0.09  | 228.1                    | 0.006            | 6.5             | 2,250.4                  | 0.00032          | 5.0             | 248.0                    | 0.0033           | -----           |
| 25       | 0.54                 | 0.09 | 1.22 | 28.1 | 35.9 | 14.8 | 5.05 | 0.11  | 59.2                     | 0.135            | 19.0            | 769.7                    | 0.00048          | 5.0             | 403.9                    | 0.0011           | 22.5            |
| 26       | 0.93                 | 0.05 | 1.29 | 28.7 | 36.5 | 14.9 | 4.96 | 0.11  | 133.4                    | 0.041            | 16.0            | -----                    | -----            | -----           | -----                    | -----            | -----           |

Based on the data in Table II, and previous experiences with heat-resistant alloys, the following broad alloy range (any balance, substantially all iron) is comprehended as one aspect of the present invention:

| C%   | Mn%  | Si% | Cr% | Ni% | Co% | W% | N%   |
|------|------|-----|-----|-----|-----|----|------|
| 0.30 | 0.02 | 0.5 | 22  | 26  | 9   | 3  | 0.01 |
| 0.95 | 1.25 | 2.0 | 32  | 42  | 26  | 16 | 0.15 |

For example, heats 11, 12 and 26, at the limits of the carbon range (carbon enhances hot strength), display excellent properties at 1800° F., 8000 p.s.i. which are rather severe conditions. The oxidation resistance of the alloy is excellent. However, the lowered carbon in heats 11 and 12 needs to be compensated for by increasing tungsten and cobalt. To avoid the expense of excessive tungsten and cobalt additions, while attaining desirable high temperature properties, the following range is inclusive of general purpose alloys contemplated herein:

| C%  | Mn%  | Si% | Cr% | Ni% | Co% | W%  | N%   |
|-----|------|-----|-----|-----|-----|-----|------|
| 0.4 | 0.02 | 0.5 | 25  | 34  | 13  | 3.0 | 0.05 |
| 0.6 | 1.25 | 2.0 | 28  | 38  | 17  | 7.0 | 0.15 |

In further explanation of the above preferred range for general purpose alloys, chromium much below 25-28% may possibly impair oxidation resistance. In fact, the lowermost limit of 22% chromium in the broad range should not be used for alloys that are to be subjected to temperatures as high as 2200° F. In this same connection, tungsten in excess of about 7%, in addition to increasing the cost of the alloy, must be used cautiously in alloy parts that will be exposed to stagnant high temperature atmospheres where catastrophic oxidation is possible.

Molybdenum is not essential as a strengthener under the present invention as will be apparent from the data in Table II. In fact, its use should be avoided, particularly in alloys for service at least as high as 2000° F., since it accentuates susceptibility to the catastrophic oxidation condition mentioned, but where it is certain that such conditions will not be encountered, then it is possible to use a limited amount of molybdenum if desired for some unique purpose. By the same token, the present alloy is also made without the need for additions of columbium, titanium or boron and like molybdenum, should be avoided in alloys for service at least as high as 2000° F.

The creep rupture data set forth herein were obtained

from castings, since alloys of this kind are generally cast. However, forgings and other wrought products are possible by appropriately lowering carbon, tungsten and cobalt.

Table III sets forth limiting creep-rupture data pertinent to design calculations for the preferred alloy under the present invention.

30

TABLE III  
Nominal Composition

| C%   | Mn%  | Si% | Cr%  | Ni%  | Co%  | W%  | N%   | Fe% |
|------|------|-----|------|------|------|-----|------|-----|
| 0.50 | 0.10 | 1.4 | 28.0 | 36.0 | 15.0 | 5.0 | 0.10 | 14- |

40

| Temp., °F | Stress (p.s.i.) for— |       |                    |        |
|-----------|----------------------|-------|--------------------|--------|
|           | Life (hours)         |       | MCR (percent/hour) |        |
|           | 100                  | 1,000 | 0.001              | 0.0001 |
| 45 1,600  | 13,500               | 9,200 | -----              | -----  |
| 1,800     | 7,000                | 4,500 | 4,400              | 3,200  |
| 1,900     | 5,100                | 3,300 | 3,300              | 2,450  |
| 2,000     | 3,500                | 2,250 | 2,300              | 1,700  |
| 2,100     | 2,250                | 1,300 | 1,300              | 950    |
| 2,200     | 1,250                | 600   | 560                | 350    |
| 2,300     | 500                  | ----- | -----              | -----  |

50

The data in Table III are based on numerous creep-rupture tests, some lasting for several thousand hours. For example, the 600 p.s.i. stress for 1000 hour life at 2200° F. is validated not only by log-log plotting of various tests and by interpolation, but also by an actual test at 2200° F. under 500 p.s.i. that endured 2868.1 hours before fracture.

For hot gas corrosion resistance, good life at 1800° F. requires that the surface metal loss be less than 0.1 inch per year. At higher temperatures greater rates are tolerated. As an example of surface stability, the above creep-rupture test at 2200° F. (Table III) showed a surface metal loss of only 0.002 inch, which is equivalent to 0.006 inch per year. As with other heat resistant alloys there is some sub-surface attack below the layer of protective scale that develops. This amounted to a total of about 0.040 inch in 1869 hours at 2200° F. or 0.19 inch per year total metal affected. Only the upper quarter of this depth was seriously affected.

Comparative tests under standardized thermal fatigue conditions show that the alloy of Table III has unusually good resistance to this type of damage, using 15 minute temperature cycles of 300 to 1800° F. Comparison with industrial alloys usually selected for thermal fatigue service were favorable. Thus, one heat of the Table III alloy

lasted 180 cycles and another, 244 cycles before failure, while the known HW (12% Cr:60% Ni) grade gave 135 cycles and the popular HT (15% Cr:35% Ni) alloy endured 158 and 202 cycles before failure.

The considerations establishing the ranges for some of the ingredients have been explained above. Silicon is essentially a deoxidizer. Nitrogen plus carbon content should not exceed 1.1% in order to avoid excess embrittlement. Manganese should not be above the range indicated, in order to avoid excessive formation of spinel-forming surface oxides which may impair oxidation resistance at very high temperatures. Calcium, zirconium, and aluminum can be used as special deoxidizers or degasifiers and these, with the usual contaminants, will not analyze more than about 0.2%. The alloy heats under the present invention can be prepared in accordance with techniques conventional to the art, and the alloys require no special heat treatment. Structural parts can either be cast directly or forged as noted, and are readily machinable.

Heat resistant alloys are reported in British Patent Nos. 640,143 and 681,247. The highest temperature for service reported in the British patents appears to be 850° C., corresponding to 1562° F. It is important to realize that the alloy of the present invention displays excellent resistance to oxidation at elevated temperatures above anything reported in the British patents. Thus, to first consider experimental heat XJ72, this analyzes as follows:

| C%   | Mn%  | Si%  | Cr%  | Ni%  | N%   | Cb%  |
|------|------|------|------|------|------|------|
| 0.48 | 0.50 | 0.58 | 26.6 | 14.1 | 0.12 | 0.99 |

This alloy has strength comparable to that of the British patents, namely, 20,000 p.s.i. at 1400° F. for 192 hours' rupture time. Two related heats that differed from XJ72 significantly only in carbon variations (XJ90 and XJ149: 0.64 and 0.66 carbon respectively) were exposed for over 3000 hours at 1900-1940° F. in an oxidizing atmosphere. Surface metal loss was 0.16-0.22 per inch per year and increasing. Similar excessive scaling rates were encountered with heats XG127 (0.31 carbon) and XG128 (0.36 carbon). In these four instances, the nickel is in the mid-range of British Patent No. 640,143 and quite close to the examples cited in British Patent No. 681,247, but the material is undesirable for service at 1900-1940° F. Additionally, solution heat treatment followed by aging is specified, but the present alloys have the properties specified in the "as cast" state. The following table sets forth the oxidation resistance of the present alloy at 2200° F.:

TABLE IV

| Heat No. | Temp., ° F. | Time, hours | Surface Dimension Change, inches per year |
|----------|-------------|-------------|-------------------------------------------|
| 17-----  | 2,200       | 1,320       | +0.020 to +0.033                          |
| 18-----  | 2,200       | 2,006       | +0.0064                                   |
| 18-----  | 2,200       | 2,368       | +0.003                                    |

NOTE: + values indicate an increased dimension because of a thin protective scale build-up.

It will be observed that the XJ90 and XJ149 alloys underwent extensive oxidation metal loss when tested at 1900-1940° F. in an oxidizing atmosphere. At a higher temperature, namely, 2200° F., an alloy under the present invention actually gained a protective scale.

United States Patent No. 2,540,107 discloses a heat-resistant alloy including nickel contents in the range 40-60%. Creep and stress rupture data for this alloy are reported at page 105 in Iron and Steel Engineer, February 1953. At 2000° F. the alloy of heat No.

212992 reported in aforesaid Iron and Steel Engineer had a duration at 2500 p.s.i. stress of 289 hours and a minimum creep rate of 0.012. The alloy of heat No. 5 reported in aforesaid Iron and Steel Engineer under the same conditions had a life of 139 hours and a creep rate of 0.041. The fundamental differences between the Iron and Steel Engineer heat No. 212992 and heat No. 5 were lower nickel for the alloy of heat No. 5 (48.9 vs. 43.1), slightly higher chromium (26.1 vs. 27.8) and about the same tungsten (6.16 vs. 5.92).

The following table contrasts the performance of three additional alloys, reported in aforesaid Iron and Steel Engineer, with an alloy of the present invention at 2300° F.

15 TABLE V  
COMPOSITION

| Heat No.                  | C    | Mn   | Si   | Ni   | Cr   | W    |
|---------------------------|------|------|------|------|------|------|
| 18-----                   |      |      |      |      |      |      |
| 2230-----                 | 0.44 | 0.80 | 1.03 | 49.3 | 29.0 | 4.96 |
| 316002-----               | 0.57 | 1.21 | 1.00 | 48.6 | 26.2 | 4.96 |
| 216997 <sup>1</sup> ----- | 0.60 | 1.43 | 1.46 | 46.8 | 26.4 | 5.14 |

## 25 CREEP AND STRESS RUPTURE DATA

| Heat No.    | Temp., ° F. | Stress, p.s.i. | Rupture time (hrs.) | MCR, percent/hr. |
|-------------|-------------|----------------|---------------------|------------------|
| 18-----     | 2,300       | 200            | 2,646.1             | 0.00022          |
| 2230-----   | 2,300       | 225            | 483                 | 0.007            |
| 316002----- | 2,300       | 130            | 2,100               | 0.0022           |
| 216997----- | 2,300       | 175            | 338                 | 0.0015           |

<sup>1</sup> Reported at Iron and Steel Engineer, February 1953, page 105.

35 It will be seen from the foregoing that under the present invention hot strength characteristics have been greatly improved in respect of a heat and corrosion-resistant alloy of the nickel-chromium type containing tungsten, and this has been accomplished by adding cobalt. The present alloy is to be distinguished from a cobalt base alloy, and is further distinguished by the absence of molybdenum, columbium and titanium. Iron is not essential as will be evident from heat No. 22 in Table II. Hence, while preferred examples of the invention have been described, these are capable of some variation and modification.

40 I claim:

45 1. A heat and corrosion resistant alloy consisting essentially of: carbon, 0.3-0.95%; silicon, 0.5-2%; nickel, 26-42%; chromium, 22-32%; tungsten, 3-16%; cobalt, 9-26%; balance, if any, essentially iron.

50 2. A heat and corrosion resistant alloy for service at temperatures at least as high as 2000° F. and, for this purpose, consisting essentially of: carbon, about 0.4-0.6%; silicon, about 0.5-2%; nickel, about 34-38%; chromium, about 25-28%; tungsten, about 3-7%; cobalt, about 13-17%; nitrogen, about 0.05-0.15%; balance, essentially iron.

55 3. A heat and corrosion resistant alloy for service at high temperatures and for this purpose, consisting essentially of: carbon, about 0.4-0.6%; silicon, about 0.5-2%; nickel, about 34-38%; chromium, about 25-28%; tungsten, about 3-7%; and cobalt, about 13-17%; balance, essentially iron.

## 60 65 References Cited in the file of this patent

## UNITED STATES PATENTS

2,206,502 Heiligman ----- July 2, 1940  
2,513,469 Franks et al. ----- July 4, 1950

## 70 FOREIGN PATENTS

640,143 Great Britain ----- July 12, 1950  
681,247 Great Britain ----- Oct. 22, 1952